

# United States Patent Office

3,305,580

Patented Feb. 21, 1967

1

3,305,580  
CYCLOALKENE-1-MERCAPTOALKANOIC ACIDS,  
ALKYL ESTERS AND METAL SALTS  
Otto A. Homberg, Woodlawn, and Ingenuin Hechen-  
bleikner and Edith H. Miller, Cincinnati, Ohio, assign-  
ors to Carlisle Chemical Works, Inc., Reading, Ohio, a  
corporation of Ohio  
No Drawing. Filed Apr. 2, 1963, Ser. No. 269,863  
13 Claims. (Cl. 260—468)

The present invention relates to the preparation of unsaturated sulfur containing carboxylic acids and to the preparation of salts and esters of such acids.

The preparation of heterocyclic compounds by the reaction of perhaloketones with thioacetic acid or thiopropionic acid is disclosed in Simmons Patent 2,911,414.

It is an object of the present invention to prepare sulfur containing unsaturated acids and esters and salts thereof which are devoid of a heterocyclic ring.

Another object is to prepare novel alkene and cyclo-  
alkene thio esters of mercaptoalkanoic acids and the esters  
and salts thereof.

A further object is to improve the heat and light sta-  
bility of halogen-containing resins.

An additional object is to provide novel stabilized vinyl  
resin compositions.

Yet another object is to provide novel synergistic sta-  
bilizers of halogen-containing resins.

Still further objects and the entire scope of applica-  
bility of the present invention will become apparent from  
the detailed description given hereinafter; it should be  
understood, however, that the detailed description and  
specific examples, while indicating preferred embodiment  
of the invention, are given by way of illustration only,  
since various changes and modifications within the spirit  
and scope of the invention will become apparent to those  
skilled in the art from this detailed description.

The novel compounds of the present invention have the  
formula  $R_1S(CH_2)_n-COOR_2$  where  $R_1$  is alkenyl, ar-  
alkenyl or cycloalkenyl in which the aliphatic or cyclo-  
aliphatic double bond is attached to the carbon atom di-  
rectly attached to the sulfur atom and  $R_2$  is hydrogen,  
alkyl, ammonium or a metal, e.g. sodium or potassium  
and  $n$  is an integer up to 10, preferably 1 or 2.

Examples of compounds within the invention are

cyclohexene-1-mercaptopropionic acid,  
cyclohexene-1-mercaptopropionic acid,  
butyl cyclohexene-1-mercaptopropionate,  
hexyl cyclohexene-1-mercaptopropionate,  
methyl cyclohexene-1-mercaptopropionate,  
methyl cyclohexene-1-mercaptopropionate,  
octadecyl cyclohexene-1-mercaptopropionate,  
octadecyl cyclohexene-1-mercaptopropionate,  
cyclohexene-1-mercaptopropionate,  
cyclohexene-1-mercaptopropionic acid,  
sodium cyclohexene-1-mercaptopropionate,  
sodium cyclohexene-1-mercaptopropionate,  
ammonium cyclohexene-1-mercaptopropionate,  
potassium cyclohexene-1-mercaptopropionate,  
cyclopentene-1-mercaptopropionic acid,  
cyclopentene-1-mercaptopropionate,  
butyl cyclopentene-1-mercaptopropionate,  
butyl cyclopentene-1-mercaptopropionate,  
hexyl cyclopentene-1-mercaptopropionate,  
octyl cyclopentene-1-mercaptopropionate,  
ethene-1-mercaptopropionic acid,  
ethene-1-mercaptopropionic acid,  
amyl ethene-1-mercaptopropionate,  
propene-1-mercaptopropionic acid,  
propene-1-mercaptopropionic acid,  
hexyl propene-1-mercaptopropionate,

2

isodecene-1-mercaptopropionic acid,  
butyl S-2-heptene mercaptoacetate,  
S-2-heptene mercaptopropionic acid,  
2-thia-3-decenoic acid,  
5 3-thia-5-ethyl-4-heptenoic acid,  
2-thia-4-ethyl-3-hexenoic acid,  
3-thia-4-undecenoic acid,  
butyl 3-thia-4-undecenoate,  
3-thia-4-eicosenoic acid,  
10 methyl 3-thia-4-eicosenoate,  
propene-2-mercaptopropionic acid,  
propene-2-mercaptopropionate,  
heptyl propene-2-mercaptopropionate,  
S-2-butene mercaptopropionic acid,  
15 S-3-pentene mercaptoacetic acid,  
butyl S-3-pentene mercaptoacetate,  
4-phenyl-2-thia-3-butenoic acid,  
3-methyl cyclohexene-1-mercaptopropionic acid,  
1-phenylethene-1-mercaptopropionic acid.

The compounds of the present invention can be pre-  
pared by heating 1 mole of a mercaptoalkanoic acid with  
1 mole, or preferably a slight excess of 1 mole, of the ap-  
propriate aldehyde or ketone and removing 1 mole of  
water. The reaction is carried out in the presence of a  
water entrainer such as a hydrocarbon solvent, e.g. tolu-  
ene, benzene, xylene or naphtha in the presence or absence  
of an acid catalyst such as hydrochloric acid, hydro-  
bromic acid, p-toluenesulfonic acid, benzenesulfonic acid  
30 or sulfuric acid.

When mercaptoacetic acid is employed as a reactant  
there are found substituted oxathiolanes as by-products.  
The desired alkene-1-mercaptopropionic acid (or cycloalkene-  
1-mercaptopropionic acid) can be separated from the 1-oxa-  
35 thiolane by adding dilute aqueous alkali such as sodium  
bicarbonate, potassium bicarbonate or ammonium hy-  
droxide. The alkene-1-mercaptopropionic acid goes into the  
aqueous layer while the oxathiolane remain in the organic  
layer. The aqueous layer can be separated and then  
40 evaporated to recover the salt of the alkene-1-mercaptop-  
propionic acid or cycloalkene-1-mercaptopropionic acid. Al-  
ternatively the separated aqueous layer can be acidified,  
e.g. with hydrochloric acid to precipitate the alkene-1-  
mercaptopropionic acid or cycloalkene-1-mercaptopropionic  
45 acid.

Since mercaptopropionic acid does not form cyclic  
compounds with the aldehydes and ketones there is no  
need to add aqueous alkali to the reaction product for  
separation purposes. However, aqueous alkali can be  
50 added to form the salt of alkene or cycloalkene-1-mer-  
captopropionic acid. The salts thus are useful for form-  
ing the free alkene and cycloalkene-1-mercaptopropionic  
acids.

The alkene and cycloalkene mercaptopropionic acid  
55 compounds can be recovered by distillation as can the  
alkylesters of alkene or cycloalkene mercaptopropionic  
(or mercaptoacetic) acids.

Distillation can also be employed to further purify the  
alkene or cycloalkene mercaptoacetic acids.

60 As starting aldehydes or ketones, there can be used  
acetaldehyde, propionaldehyde, butyraldehyde, valeralde-  
hyde, isovaleraldehyde, caprylaldehyde, 2-ethyl-butyral-  
dehyde, stearaldehyde, phenylpropionaldehyde, acetone,  
methyl ethyl ketone, methyl propyl ketone, methyl butyl  
ketone, methyl isobutyl ketone, stearanone, diethyl ke-  
tone, dipropyl ketone, ethyl propyl ketone, acetophenone,  
65 propiophenone, cyclopentanone, cyclohexanone, 2-meth-  
yl cyclohexanone, methyl amyl ketone, and isodecalde-  
hyde.

70 The compounds of the present invention, especially the  
free acids and the alkyl esters are useful as stabilizers for  
halogen containing minerals particularly when used with

tin compounds such as dialkyltin oxide and dialkyltin acylates.

The stabilizers of the present invention can be used with halogen containing vinyl and vinylidene resins in which the halogen is attached directly to the carbon atoms. Preferably, the resin is a vinyl halide resin, specifically, a vinyl chloride resin. Usually, the vinyl chloride resin is made from monomers consisting of vinyl chloride alone or a mixture of monomers comprising at least 70% vinyl chloride by weight. When vinyl chloride copolymers are stabilized, preferably the copolymer of vinyl chloride with an ethylenically unsaturated compound copolymerizable therewith contains at least 10% of polymerized vinyl chloride.

As the chlorinated resin there can be employed chlorinated polyethylene having 14 to 75%, e.g., 27%, chlorine by weight. Polyvinyl chloride, polyvinylidene chloride, polyvinyl bromide, polyvinyl fluoride, copolymers of vinyl chloride with 1 to 90%, preferably 1 to 30%, of a copolymerizable ethylenically unsaturated material such as vinyl acetate, vinyl butyrate, vinyl benzoate, vinylidene chloride, diethyl fumarate, diethyl maleate, other alkyl fumarates and maleates, vinyl propionate, methyl acrylate, 2-ethylhexyl acrylate, butyl acrylate and other alkyl acrylates, methyl methacrylate, ethyl methacrylate, butyl methacrylate and other alkyl methacrylates, methyl alpha chloroacrylate, styrene, trichloroethylenes, vinyl ethers such as vinyl ethyl ether, vinyl chloroethyl ether and vinyl phenyl ether, vinyl ketones such as vinyl methyl ketone and vinyl phenyl ketone, 1-fluoro-1-chloroethylene, acrylonitrile, chloroacrylonitrile, allylidene diacetate and chloroallylidene diacetate. Typical copolymers include vinyl chloride-vinyl acetate (96:4 sold commercially as VYNW), vinyl chloride-vinylacetate (87:13), vinyl chloride-vinyl acetate-maleic anhydride (86:13:1), vinyl chloride-vinylidene chloride (95:5), vinyl chloride-diethyl fumarate (95:5), vinyl chloride trichloroethylene (95:5), vinyl chloride-2-ethylhexyl acrylate (80:20).

The stabilizers of the present invention can be incorporated with the resin by admixing in an appropriate mill or mixer or by any of the other well-known methods which provide for uniform distribution throughout the resin compositions. Thus, mixing can be accomplished by milling on rolls at 100-160° C.

In addition to the novel stabilizers there can also be incorporated with the resin conventional additives such as plasticizers, pigments, fillers, dyes, ultraviolet light absorbing agents, densifying agents and the like.

If a plasticizer is employed, it is used in conventional amount, e.g., 30 to 150 parts per 100 parts of resin. Typical plasticizers are di-2-ethyl-hexyl phthalate, dibutyl sebacate, dioctyl sebacate, tricresyl phosphate.

Examples of suitable tin compounds for use as stabilizers with the compounds of the present invention are dibutyltin oxide, dibutyltin dilaurate, dioctyltin oxide, dioctyltin dilaurate.

The compounds of the present invention are normally used in an amount of 0.01 to 10% by weight of the resin.

The tin compounds are also normally used in an amount of 0.01 to 10% by weight of the resin. More preferably 0.2 to 5% of the tin compound and 0.2 to 5% of the alkene or cycloalkene mercaptoalkanoic acid (or alkyl ester thereof) of the present invention are used based on the weight of the resin.

Unless otherwise indicated all parts and percentages are by weight.

The alkene and cycloalkene group containing compounds of the present invention can also be prepared by forming a thioacetal or thionketal from 2 moles of mercaptoacetic acid or mercaptopropionic acid or an alkyl ester thereof and 1 mole of the appropriate aldehyde or ketone and then heating to remove 1 mole of mercaptoacetic acid.

#### Example 1

1 mole of mercaptopropionic acid and 1.1 mole of

cyclohexanone were refluxed in toluene with removal of water (the reactants together equalled 80% by weight of the total mixture) until 18 grams of water were obtained. The product was then distilled and cyclohexene-1-mercaptopropionic acid was recovered as a yellow liquid having an  $n_D^{23}$  1.5319 and a B.P. of 142-145° C. at 0.5 mm. Hg. The product had the formula



#### Example 2

The procedure of Example 1 was repeated replacing the mercaptopropionic acid by 1 mole of butyl mercaptopropionate. The product was butyl cyclohexene-1-mercaptopropionate, a colorless liquid having an  $n_D^{20}$  1.4983, having a B.P. of 133° C. at 0.5 mm. Hg and having the formula



#### Example 3

The procedure of Example 1 was repeated replacing the mercaptopropionic acid by 1 mole of butyl mercaptoacetate. The product was butyl cyclohexene-1-mercaptopacetate, a colorless liquid having an  $n_D^{20}$  of 1.5022 and having a B.P. of 133-140° C. at 1.9 mm. Hg.

#### Example 4

The procedure of Example 1 was repeated but the reactants employed were 1 mole of butyl mercaptoacetate and 1.1 mole of methyl amyl ketone. The product was butyl S-2-heptene mercaptoacetate, a colorless liquid having an  $n_D^{18}$  1.4739, a B.P. of 117-126° C., at 0.3 mm. and having the formula



#### Example 5

To a mixture of 1 mole of mercaptopropionic acid and 1.1 mole of cyclopentanone in toluene there was added 3 grams of p-toluenesulfonic acid as a catalyst. The reactants equalled 80% by weight of the toluene. The mixture was refluxed with removal of water until 18 grams thereof were obtained. The product was then washed with dilute aqueous sodium bicarbonate, the toluene removed by distillation and cyclopentene-1-mercaptopropionic acid recovered as a yellow solid M.P. 33-35° C.

#### Example 6

The procedure of Example 1 was repeated replacing the cyclohexanone by 1.1 mole of isodecaldehyde. The product was isodecene-1-mercaptopropionic acid, a colorless liquid having an  $n_D^{20}$  1.4878, a B.P. of 163-173° C., at 0.4 mm. Hg and having the formula



#### Example 7

The procedure of Example 5 was repeated replacing the cyclopentanone by 1.1 mole of methyl amyl ketone. The product was S-2-heptene mercaptopropionic acid, a light brown solid melting at about 37° C. and having the formula



#### Example 8

1 mole of mercaptoacetic acid and 1.1 mole of caprylic aldehyde were refluxed in toluene with removal of water

until 18 grams of water were obtained. The reactants together equalled 80% by weight of the total mixture. The product was then treated with an equal weight of dilute (10%) aqueous sodium bicarbonate and the water layer containing the sodium salt of 2-thia-3-decenoic acid separated from the organic layer. The water layer was then neutralized with hydrochloric acid to separate the free 2-thia-3-decenoic acid, from the water. After removal of the aqueous layer the 2-thia-3-decenoic acid having the formula  $\text{CH}_3(\text{CH}_2)_5\text{CH}=\text{CHSCH}_2\text{COOH}$  was recovered as a colorless liquid having an  $n_{\text{D}}^{20}$  1.4919 and a boiling point of 130-138° C. at 0.5 mm. Hg.

*Example 9*

The procedure of Example 1 was repeated replacing the cyclohexanone by 1.1 mole of 2-ethylbutyraldehyde. The product was 3-thia-5-ethyl-4-heptenoic acid, a deep yellow liquid having an  $n_D^{21}$  1.5015, a B.P. of 132–138° C. at 0.3 mm. and the formula



*Example 10*

The procedure of Example 1 was repeated using as the reactants 1 mole of mercaptoacetic acid and 1.1 mole of 2-ethylbutyraldehyde. The product was 2-thia-4-ethyl-3-hexenoic acid, a colorless liquid having an  $n_D^{20}$  1.5008 and a B.P. of 130–140° C. at 2 mm. Hg.

*Example 11*

The procedure of Example 5 was followed replacing the cyclopentanone by 1.1 mole of caprylaldehyde. The product was 3-thia-4-undecenoic acid, a yellow liquid having  $n_D^{20}$  1.4898 and a B.P. of 147–150° C. at 0.3 mm. Hg.

*Example 12*

The procedure of Example 1 was followed employing as the reactants 1 mole of butyl mercaptopropionate and 1.1 mole of caprylaldehyde. The product was butyl 3-thia-4-undecenoate, a pale yellow liquid having an  $n_D^{22}$  1.4731 and a B.P. of 136–146 ° C. at 1 mm. Hg.

*Example 13*

100 parts of Geon 101EP (vinyl chloride homopolymer) was mixed with 0.37 part dibutyltin oxide and 0.30 part of cyclohexane-1-mercaptopropionic acid to form a heat stable product.

*Example 14*

Example 13 was repeated but 50 parts of dioctyl phthalate was included in the composition. The product was heat stable.

What is claimed is:

1. A compound having the formula  $R_1S(CH_2)_nCOOR_2$  where  $R_1$  is cycloalkenyl in which the double bond is on the carbon atom adjacent to the sulfur atom,  $R_2$  is selected from the group consisting of hydrogen, alkyl and a metal and  $n$  is an integer of at least 1.

5 2. A compound according to claim 1 wherein  $R_2$  is lower alkyl.

10 3. Cycloalkene-1-mercaptoalkanoic acids wherein the cycloalkene group has 5 to 6 carbon atoms and the mercaptoalkanoic group has 2 to 3 carbon atoms.

15 4. Cyclohexene-1-mercaptoalkanoic acids wherein the mercaptoalkanoic group has 2 to 3 carbon atoms.

19 5. Cyclohexene-1-mercaptoacetic acid.

25 6. Cyclohexene-1-mercaptopropionic acid.

20 7. Cyclopentene-1-mercaptoalkanoic acids wherein the mercaptoalkanoic group has 2 to 3 carbon atoms.

20 8. Alkyl esters of cycloalkene-1-mercaptoalkanoic acids wherein the cycloalkene group has 5 to 6 carbon atoms and the mercaptoalkanoic group has 2 to 3 carbon atoms wherein the alkyl group has 1 to 18 carbon atoms.

25 9. A compound according to claim 8 where the alkyl is lower alkyl.

25 10. Alkyl esters of cyclohexene-1-mercaptoalkanoic acids wherein the mercaptoalkanoic group has 2 to 3 carbon atoms wherein the alkyl group has 1 to 18 carbon atoms.

30 11. A compound according to claim 10 where the alkyl is lower alkyl.

30 12. Alkyl esters of cyclohexene-1-mercaptopropionic acid wherein the alkyl group has 1 to 18 carbon atoms.

35 13. A compound according to claim 12 where the alkyl is lower alkyl.

5 References Cited by the Examiner

UNITED STATES PATENTS

3,026,349 3/1962 Celmer ----- 260—516 X

0 FOREIGN PATENTS

0 839,561 6/1960 Great Britain.

0 OTHER REFERENCES

5 Voronkena et al.: "J. Gen. Chem. (U.S.S.R.)" vol. 32 (1962), pp. 3877—3882.

5 Shriner et al.: "J. Am. Chem. Soc." vol. 61 (1939), pp. 2001—2003.

0 Kharasch: "Organic Sulfur Compounds," vol. 1 (1961), page 134.

0 LORRAINE A. WEINBERGER, Primary Examiner.

0 R. K. JACKSON, Assistant Examiner.